# EUROPEAN PATENT SPECIFICATION

(11) **EP 3 215 287 B1**
(45) Date of publication and mention of the grant of the patent: **08.04.2020**
(21) Application number: 14793190.1
(22) Date of filing: 05.11.2014
(51) Int. Cl.: B22D 11/124, C23C 22/68, C23F 11/18, C23F 15/00

(54) **METHOD TO CONTROL CORROSION IN CONTINUOUS CASTERS**
VERFAHREN ZUR STEUERUNG DER KORROSION IN STRANGSGUSSVORRICHTUNGEN
PROCÉDÉ DE LUTTE CONTRE LA CORROSION DANS UNE COULÉE EN CONTINU

(43) Date of publication of application: 13.09.2017
(73) Proprietor: Ecolab USA Inc., St. Paul, MN 55102 (US)
(72) Inventor: JOHNSON, Donald, NL-2342 BV Oegstgeest (NL); ROCA, Laia, More, NL-2342 BV Oegstgeest (NL); MYERS, Craig, NL-2342 BV Oegstgeest (NL); SERRANO, Paloma Lopez, NL-2342 BV Oegstgeest (NL)
(74) Representative: Michalski Hüttermann & Partner Patentanwälte mbB
(86) International application number: PCT/EP2014/073826
(87) International publication number: WO 2016/070914

(56) References cited:
- WO-A2-03/106074
- DE-A1- 3 317 126
- A. D. Pomogailo ET AL: "Monomeric and Polymeric Carboxylic Acids", Macromolecular Metal Carboxylates and Their Nanocomposites, 1 January 2010 (2010-01-01), XP055489755, Berlin, Heidelberg ISBN: 978-3-642-10574-6 Retrieved from the Internet: URL:https://www.springer.com/cda/content/d ocument/cda_downloaddocument/9783642105739 -c1.pdf?SGWID=0-0-45-993442-p173959909 [retrieved on 2018-07-03]

## Description

The present invention deals with continuous casters which are used in steel production, especially the control of the pH in those continuous casters.

During the production of steel in continuous casters, in most applications water is sprayed to cool down the steel being molded. Usually almost all parts within the spray chamber are in contact with sprayed water or vapor which creates a highly corrosive environment due to the high temperature and not always optimal contact of water with the metal surfaces.

Under these harsh conditions, a good water quality control is critical to minimize corrosion of steel parts. Corrosion ultimately leads not only to high costs of equipment replacement but, more important, to extreme losses due to production down-time.

Poor control of the water quality may also have a dramatic impact on the steel production quality. If the spray nozzles plug due to formation of mineral scale and/or accumulation of deposits, the cooling profile of the strand could deteriorate and alter the quality of the final produced product.

One critical water quality parameter to control is pH: Low pH could result in high corrosion of carbon steel, while high pH could result in uncontrolled formation of mineral scale. The pH should therefore be maintained in all areas of the spray chamber at the right pH at which the corrosion and scale inhibitor program can be effective.

For most applications the spray chamber environment can be subdivided into three zones: 1. the fully submerged zone; 2. the spray wetted zone; and 3. the condensate wetted zone. The corrosion challenges in these three zones are distinctly different. In the fully submerged and spray wetted zones, the aqueous composition is substantially that of the bulk water, including all water components and inhibitors. In the condensate wetted zone, the water composition is defined by the volatility of the components of the water producing the vapors. Since inhibitors and inorganic ions are essentially nonvolatile, and acidic gasses such as CO₂, HCl and HF are fairly volatile, the composition, and resulting corrosiveness are largely defined by the acidic gasses.

When the pH in spray chambers is controlled, this is typically done by adding sodium bicarbonate, sodium carbonate, or sodium hydroxide based on a given pH set point measured in the bulk water. This method is used to maintain a non-corrosive pH and provide additional alkalinity to the water that would be available to neutralize the acid locally formed by the mold powder in the upper zone of the spray chamber. However, at the range of pH values typically used in spray chambers, the addition of these species in excess can produce undesirable scaling conditions in the bulk water, placing limits on how much buffering capacity can be added by the use of these agents.

DE 33 17 126 A1 refers to a process to avoid acid caused corrosion in a caster for the production of steel, wherein to spray water a base solution and a dispersant is added.

WO 03/106074 A2 refers to a process for reducing the corrosiveness of cooling or process water, in which the pH is reduced by the addition of acids, at least one water-soluble salt with a buffering effect being added to the cooling or process water.

In most applications and steel-making processes a problem that is widely observed is the formation of hydrofluoric acid, a volatile, and corrosive substance. Hydrofluoric acid is a relatively and very volatile acid with a pKa of ∼4 and an Henry's law constant of 3.2 at 40° C. The most volatile form of fluoride is the protonated form with a Henry's law constant of 3.2 at 40° C.

The mold powder used during production produces said hydrofluoric acid when contacting water. If the cooling water is sufficient basic, then the alkalinity in the cooling water will neutralize the acidity, and the flouride produced will be predominantly in the ionized nonvolatile F⁻ form, but, if the level is not sufficient for a complete neutralization, once the buffering capacity has been exhausted, the pH will rapidly drop down to 2-4, particularly in the high heat flux areas where mold powders are pyrolyzed into fluoride species. At these pH levels, fluoride will be converted into the undissociated HF species, which is quite volatile. This will facilitate acidification of vapors produced by contact with hot metals. When these vapors condense, extensive corrosion can occur then in the condensate zone, especially on carbon steel, low alloy and galvanized steels. Corrosion caused by acidic conditions in spray wetted zones is also a major concern and is typically found in metal parts directly below the mold powder addition point. At lower levels in the chamber, the acid corrosion intensity is milder due to the neutralization of acid when mixing with the bulk water where alkalinity is still available.

It is therefore a constant need to improve the water treatment in continuous casters in steel mills, especially concerning the pH control. This object is met by the buffer system of claim 1.

Accordingly, a buffer system for the production of steel, by which water or aqueous solution can be sprayed by a caster comprising a plurality of water sprayers on the steel being molded in the caster, comprising:
a) a primary buffer system buffering the water or aqueous solution of at least one of said water sprayers, which comprises one or more salts selected from the group of carbonate salts, bicarbonate salts, hydroxy salts; and
b) a secondary buffer system buffering the water or aqueous solution of the at least one of said water sprayers, whereby said secondary buffer system is different from the primary buffer system and said buffer comprises one or more salts from acids selected from the group of phosphorous acid, carboxylic acids, carboxylic/phosphoric acids, phosphinic acids, amino acids, or mixtures, or conjugate base salts thereof, wherein the carboxylic acids are selected from citric acid, succinic acid, adipic acid, sebacic acid, malic acid, having a pKa from ≥ 4.5 to ≤ 7.5; and whereby the solubility of the salt of the acid of the secondary buffer system in deionized water at 25°C is ≥ 100g/l;
c) whereby the caster furthermore comprises at least one pH-meter, whereby the pH-meter of the caster, by which the pH of said aqueous solution, which has cooled the molded steel, is measured and wherein the flow control device of the caster controlls and adapts the secondary buffer upon the measurement of the pH.

By doing so it is for many applications in the present invention possible to reduce the content of corrosive gasses in the condensate zone without increasing the pH and carbonate load of the bulk water into an excessively scaling range. This is done by adding an additional secondary buffer with a pKa in the described range. This gives the water additional resistance to local pH excursions in that pH range and helps to prevent the formation of volatile HF in areas of water vaporization and mold powder pyrolysis.

It has been found that such a caster has for a wide range of applications within the present invention at least one of the following advantages:
- By differentiating between a primary and a secondary buffer system it is possible to react to changes within the caster without overly increasing the scaling tendency, thus minimizing the risk of spray lines and nozzles being deteriorated by precipitation of inorganic salts
- The system can easily be installed on existing casters and does not require a sophisticated set-up

Once the buffer capacity is reduced or exhausted addition of a small amount of acidic substances by, for example, pyrolysis of mold powders, can produce a dramatic reduction in pH. This not only causes the bulk water and spray to become more corrosive, but also facilitates the volatilization of corrosive gasses into the vapor phase. Upon condensation, these vapors produce a very corrosive environment.

It should be noted that although separating the addition of the secondary buffer into the spray streams is preferred, this is not limiting and it is also recognized that the secondary buffer can provide benefits when added at other points in the system.

It should be noted that in the sense of the present invention the term "buffer" shall explicitly also include any basic or alkali substance that can be used to neutralize acids, i.e. also hydroxy salts which in another context might not usually be referred to as buffers.

According to a preferred embodiment of the present invention, the primary buffer system is adapted to buffer the water or aqueous solution so that after buffering the (then) aqueous solution has a total buffer concentration of ≥10 ppm to ≤1000 ppm.

The term "buffer concentration" in the sense of the present invention especially means and/or includes for a given substance both any acidic and basic forms, i.e. for citrate both citric acid and (in case that sodium is the counter-ion) the mono, bi, and trisodium citrate, in case they are present in the solution. The term "buffer concentration" is also intended to be related to the representative buffers, e.g. in terms of the primary buffer system the buffers that belong to said primary buffer system.

The term "total buffer concentration" in the sense of the present invention especially means and/or includes the total buffer concentration of all appropriate and relating substances present in the solution.

The above concentration has been found in many applications to be a good compromise between adequate buffering and avoiding excessive scaling conditions in the caster. Preferably after buffering the aqueous solution has a buffer concentration of ≥ 25 ppm to ≤ 750 ppm, more preferred ≥ 50 ppm to ≤ 600 ppm and most preferred ≥100 ppm to ≤500 ppm

According to a preferred embodiment of the present invention, the secondary buffer system is adapted to buffer the water or aqueous solution so that after buffering the (then) aqueous solution has a total buffer concentration of ≥10 ppm to ≤1000 ppm.

The above concentration has been found in many applications to be a good compromise between adequate buffering and avoiding excessive scaling conditions in the caster. Preferably after buffering the aqueous solution has a buffer concentration of ≥ 25 ppm to ≤ 750 ppm, more preferred ≥ 50 ppm to ≤ 600 ppm and most preferred ≥100 ppm to ≤500 ppm

According to a preferred embodiment of the present invention, the secondary buffer system comprises at least one organic buffer.

The term "organic buffer" in the sense of the present invention especially means and/or includes any acid or salts thereof which does contain carbon in a different form than carbonate and/or bicarbonate, with a pKa in the claimed range. It should be noted that this may be the second protonation step for multiacids (such as e.g. citric acid with pKa's of 3.13, 4.76 and 6.39).

The secondary buffer system comprises at least one salt of a acid whereby the solubility of the salt in deionized water at 25°C is ≥ 100g/l, preferably >200g/l. This has been found to be advantageous for many applications in the art.

According to a preferred embodiment of the present invention, said salt of a acid is a potassium and/or sodium salt.

According to a preferred embodiment of the present invention the secondary buffer system comprises at least one acid whereby the solubility of the calcium or magnesium salt of the acid in deionized water at 25°C is ≥ 0.7g/l, preferably ≥ 1 g/l more preferred ≥ 0 2g/l. This has been found to be advantageous for many applications in the art, because by doing so, the buffering capacity of the water can be increased without increasing the scaling potential of the cooling water.

The secondary buffer system comprises one or more salts from acids selected from the group of phosphorous acid, carboxylic acids, carboxylic/phosphoric acids, phosphinic acids, amino acids, polymers comprising acidic functionalities, or mixtures or conjugate base salts thereof.

Preferred polymers comprising acidic functionalities are poly(meth)acrylic acids, poly(meth)acrylic acid /(meth)acrylamide copolymers or mixtures thereof. These polymers are especially preferred due to their tendency to either suppress or not overly support microbial growth.

The secondary buffer system comprises one or more salts from acids selected from the group of phosphorous acid, citric acid, succinic acid, adipic acid, sebacic acid, malic acid or mixtures or conjugate base salts thereof.

According to a preferred embodiment of the present invention the caster furthermore comprises at least one pH-meter by which the pH of said aqueous solution which has cooled the molded steel in the upper zone of the spray chamber can be measured and a flow control device by which the secondary buffer system can be controlled and adapted upon the measurement of the pH.

This can according to a preferred embodiment of the present invention e.g. be achieved by using a sampling device by which aqueous buffered solution which has cooled the molded steel can be collected and its pH be measured.

By doing so it has been found out in most applications of the present invention that it is possible to cope for sudden changes/drops in pH which are then matched with an increase of secondary buffer.

The amount of secondary buffer can then be increased or decreased depending on the need. This can be done e.g. by having a valve or a pump delivering high concentrated secondary buffer solution into the aqueous solution or by other devices or solution pertinent to those skilled in the art of the field of the invention.

According to a preferred embodiment of the present invention the secondary buffer is increased when the measured pH is below a certain threshold. This threshold preferably is a fixed pH and is preferably between ≥6.0 to ≤8.5.

According to a preferred embodiment of the present invention the secondary buffer is increased when difference in pH between the average pH of the water or aqueous solution, either amongst all sprayers or for at least one preselected sprayer and the measured pH in the upper zone of the spray chamber is over a certain threshold.

It has been found out to be advantageous if said threshold (= pH difference) is somewhat between ≥0.7 ≤2.5 pH units . This is for most applications a good compromise between the desire to use additional secondary buffer only when needed and the desire to achieve a beneficial effect from the presence of said secondary buffer system.

Although separate addition of the acid buffer to the sprayer water is preferred, it is also recognized that the acid buffer can be added at any point in the system, and through intermixing of the recirculating water will provide benefits in the form of increased resistance to pH suppression.

The aforementioned components, as well as the claimed components and the components to be used in accordance with the invention in the described embodiments, are not subject to any special exceptions with respect to their size, shape, material selection and technical concept such that the selection criteria known in the pertinent field can be applied without limitations.

### BRIEF DESCRIPTION OF THE DRAWINGS

Additional details, characteristics and advantages of the object of the invention are disclosed in the subclaims and the following description of the respective figures--which in an exemplary fashion--show several preferred embodiments of the present invention. Such embodiments do not necessarily represent the full scope of the invention, however, and reference is made therefore to the claims and herein for interpreting the scope of the invention.

In the drawings:
Fig. 1 is a schematic illustration of a first embodiment of the present invention and
Fig. 2 is a diagram showing the changes in pH in a conventional caster line over time.

Fig. 1 shows a very schematic illustration of a first embodiment of the present invention. As can be seen in Fig. 1, steel is made in a steel mill 1. The hot liquid steel 15 enters the spray chamber at the outlet 10 and is then guided over a set of rolls 20 where it is formed and cooled down.

Furthermore there are several sprayers, schematically represented as 40 to 43 which cool the steel with aqueous solution. These sprayers are equipped with a delivery system for primary buffer and a delivery system for secondary buffer, both are not shown in Fig. 1. This delivery can be achieved e.g. by valves or pumps.

To control the secondary buffer system, a sampling device 50 is located under the upper segments. Said sampling device 50 collects water from the upper sprays and measures its pH. Alternatively, the pH can be directly measured without a sampling device. Once the pH deviates from a certain threshold, the secondary buffer is increased by the delivery system.

The embodiment of Fig. 1 is highly schematic and it is apparent to the skilled person in the art that other applications are easily possible. So it could be that there is more than one sampling device and different sprayers are controlled by different sampling devices (either that each sprayer has its own device or that a device controls several sprayers).

Fig. 2 is a diagram showing the changes in pH in a conventional steel caster spray chamber over time. In this caster only an inorganic buffer sodium bicarbonate buffer with pH control of the bulk water 8.7 was used. The pH of the spray water of the upper zone which had passed the steel (equivalent to the water collected with the sampling device 50 in Fig. 1) was continuously measured over several days.

It is apparent from Fig. 2 that although there is constant buffering, the pH can change variably and even go down to rather acidic conditions of 4 to 5. At this pH usually quite drastic corrosion can be observed.

According to preferred embodiments of the present invention, the secondary buffer in the sprayers located in the upper zone of the spray chamber would be increased once the pH of the water collected with the sampling device deviates too much from the pH of the bulk water. Depending on the actual application this could either be set that once the pH goes under an absolute value (e.g. 8.0 or 7.5) then the dosage of secondary buffer is initiated or if the pH difference rises over 0.7 or 1.0.

## Claims

1. A buffer system for the production of steel, by which water or aqueous solution can be sprayed by a caster comprising a plurality of water sprayers on the steel being molded in the caster, comprising:
a) a primary buffer system buffering the water or aqueous solution of at least one of said water sprayers, which comprises one or more salts selected from the group of carbonate salts, bicarbonate salts, hydroxy salts; and
b) a secondary buffer system buffering the water or aqueous solution of at least one of said water sprayers, whereby said secondary buffer system is different from the primary buffer system and said buffer comprises one or more salts from acids selected from the group of phosphorous acid, carboxylic acids, carboxylic/phosphoric acids, phosphinic acids, amino acids, or mixtures, or conjugate base salts thereof, wherein the carboxylic acids are selected from citric acid, succinic acid, adipic acid, sebacic acid, malic acid, having a pKa from ≥ 4.5 to ≤ 7.5; and whereby the solubility of the salt of the acid of the secondary buffer system in deionized water at 25°C is ≥ 100g/l;
whereby the caster furthermore comprises at least one pH-meter, whereby the pH-meter of the caster, by which the pH of said aqueous solution, which has cooled the molded steel, is measured and wherein the flow control device of the caster controls and adapts the secondary buffer upon the measurement of the pH.

2. The buffer system according to claim 1 whereby the secondary buffer system comprises at least one organic buffer.

3. A method for the production of steel, wherein a buffer system according to any of claims 1 to 2, is used for buffering the water or aqueous solution of at least one of said water sprayers, whereby the caster furthermore comprises at least one pH-meter, whereby the pH of said aqueous solution, which has cooled the molded steel, is measured with a pH-meter of the caster, and wherein the secondary buffer is controlled and adapted by the flow control device of the caster upon the measurement of the pH.

4. The method according to claim 3, whereby the secondary buffer is increased when the measured pH is below a certain threshold.

5. The method according to claim 3 or 4, whereby the secondary buffer is increased when difference in pH between the average pH of the water or aqueous solution, either amongst all sprayers or for at least one preselected sprayer and the measured pH is over a certain threshold.

6. The method according to any of the claims 3 to 5, whereby the primary buffer system after buffering the (then) aqueous solution has a total buffer concentration of ≥10 ppm to ≤1000 ppm.

7. The method according to any of the claims 3 to 6, whereby the secondary buffer system after buffering the (then) aqueous solution has a total buffer concentration of ≥10 ppm to ≤1000 ppm.

## Patentansprüche

1. Puffersystem für die Herstellung von Stahl, durch das Wasser oder eine wässrige Lösung von einer Stranggussanlage, die mehrere Wassersprühgeräte umfasst, auf den in der Stranggussanlage geformten Stahl gesprüht werden kann, Folgendes umfassend:
a) ein primäres Puffersystem, das das Wasser oder die wässrige Lösung von wenigstens einem der Wassersprühgeräte puffert, das ein oder mehrere Salze umfasst, die aus der Gruppe von Carbonatsalzen, Bicarbonatsalzen, Hydroxysalzen ausgewählt sind; und
b) ein sekundäres Puffersystem, das das Wasser oder die wässrige Lösung von wenigstens einem der Wassersprühgeräte puffert, wodurch sich das sekundäre Puffersystem von dem primären Puffersystem unterscheidet und der Puffer ein oder mehrere Salze aus Säuren umfasst, die aus der Gruppe der Phosphorsäuren Carbonsäuren, Carbon-/ Phosphorsäuren, Phosphinsäuren, Aminosäuren oder Gemischen oder konjugierten Basensalzen davon ausgewählt sind, wobei die Carbonsäuren aus Zitronensäure, Bernsteinsäure, Adipinsäure, Sebacinsäure, Äpfelsäure mit einem pKa von ≥ 4,5 bis ≤ 7,5 ausgewählt sind; und wodurch die Löslichkeit des Salzes der Säure des sekundären Puffersystems in entionisiertem Wasser bei 25°C ≥ 100 g/l ist;
wodurch die Stranggussanlage ferner wenigstens ein pH-Meter umfasst, wodurch das pH-Meter der Stranggussanlage, durch das der pH-Wert der wässrigen Lösung, die den geformten Stahl abgekühlt hat, gemessen wird, und wobei die Durchflusssteuervorrichtung der Stranggussanlage bei der Messung des pH-Werts den sekundären Puffer steuert und anpasst.

2. Puffersystem nach Anspruch 1, wodurch das sekundäre Puffersystem wenigstens einen organischen Puffer umfasst.

3. Verfahren für die Herstellung von Stahl, wobei ein Puffersystem nach einem der Ansprüche 1 bis 2, zum Puffern des Wassers oder der wässrigen Lösung von wenigstens einem der Wassersprühgeräte verwendet wird, wodurch die Stranggussanlage ferner wenigstens ein pH-Meter umfasst, wodurch der pH-Wert der wässrigen Lösung, die den geformten Stahl abgekühlt hat, mit einem pH-Meter der Stranggussanlage gemessen wird, und wobei der sekundäre Puffer durch die Durchflusssteuervorrichtung der Stranggussanlage bei der Messung des pH-Werts gesteuert und angepasst wird.

4. Verfahren nach Anspruch 3, wodurch der sekundäre Puffer gesteigert wird, wenn der gemessene pH-Wert unter einem bestimmten Schwellenwert liegt.

5. Verfahren nach Anspruch 3 oder 4, wodurch der sekundäre Puffer gesteigert wird, wenn eine pH-Wert-Differenz zwischen dem durchschnittlichen pH-Wert des Wassers oder der wässrigen Lösung, entweder unter allen Sprühgeräten oder für wenigstens ein vorausgewähltes Sprühgerät, und dem gemessenen pH-Wert über einem bestimmten Schwellenwert liegt.

6. Verfahren nach einem der Ansprüche 3 bis 5, wodurch das primäre Puffersystem nach dem Puffern der (dann) wässrigen Lösung eine Gesamtpufferkonzentration von ≥ 10 ppm bis ≤ 1000 ppm aufweist.

7. Verfahren nach einem der Ansprüche 3 bis 6, wodurch das sekundäre Puffersystem nach dem Puffern der (dann) wässrigen Lösung eine Gesamtpufferkonzentration von ≥ 10 ppm bis ≤ 1000 ppm aufweist.

## Revendications

1. Système tampon pour la production d'acier, par lequel de l'eau ou une solution aqueuse peut être pulvérisée par une machine de coulée comprenant une pluralité de pulvérisateurs d'eau sur l'acier en cours de moulage dans la machine de coulée, comprenant :
a) un système tampon primaire tamponnant l'eau ou la solution aqueuse d'au moins l'un desdits pulvérisateurs d'eau, lequel comprend un ou plusieurs sels choisis dans le groupe des sels de carbonate, des sels de bicarbonate, des sels d'hydroxyde ; et
b) un système tampon secondaire tamponnant l'eau ou la solution aqueuse d'au moins l'un desdits pulvérisateurs d'eau, ledit système tampon secondaire étant différent du système tampon primaire et ledit tampon comprenant un ou plusieurs sels issus d'acides choisis dans le groupe constitué de l'acide phosphoreux, des acides carboxyliques, des acides carboxyliques/phosphoriques, des acides phosphiniques, des acides aminés, ou de mélanges ou sels de base conjuguée de ceux-ci, les acides carboxyliques étant choisis parmi l'acide citrique, l'acide succinique, l'acide adipique, l'acide sébacique, l'acide malique, ayant un pKa de ≥ 4,5 à ≤ 7,5 ; et la solubilité du sel de l'acide du système tampon secondaire dans l'eau désionisée à 25 °C étant ≥ 100 g/L ;
la machine de coulée comprenant en outre au moins un pH-mètre, par lequel le pH de ladite solution aqueuse, laquelle a refroidi l'acier moulé, est mesuré, et le dispositif de régulation de débit de la machine de coulée régulant et adaptant le tampon secondaire lors du mesurage du pH.

2. Système tampon selon la revendication 1 selon lequel le système tampon secondaire comprend au moins un tampon organique.

3. Procédé de production d'acier, dans lequel un système tampon selon l'une quelconque des revendications 1 à 2 est utilisé pour tamponner l'eau ou la solution aqueuse d'au moins l'un desdits pulvérisateurs d'eau, la machine de coulée comprenant en outre au moins un pH-mètre, le pH de ladite solution aqueuse, qui a refroidi l'acier moulé, étant mesuré à l'aide d'un pH-mètre de la machine de coulée, et le tampon secondaire étant régulé et adapté par le dispositif de régulation de débit de la machine de coulée lors du mesurage du pH.

4. Procédé selon la revendication 3, selon lequel le tampon secondaire est augmenté lorsque le pH mesuré est inférieur à un certain seuil.

5. Procédé selon la revendication 3 ou 4, selon lequel le tampon secondaire est augmenté lorsque la différence de pH entre le pH moyen de l'eau ou de la solution aqueuse, soit parmi tous les pulvérisateurs, soit pour au moins un pulvérisateur présélectionné, et le pH mesuré, excède un certain seuil.

6. Procédé selon l'une quelconque des revendications 3 à 5, selon lequel le système tampon primaire, après avoir tamponné (ce qui constituait alors) la solution aqueuse, présente une concentration totale de tampon de ≥ 10 ppm à ≤ 1000 ppm.

7. Procédé selon l'une quelconque des revendications 3 à 6, selon lequel le système tampon secondaire, après avoir tamponné (ce qui constituait alors) la solution aqueuse, présente une concentration totale de tampon de ≥ 10 ppm à ≤ 1000 ppm.
